

June 12, 1928.

1,673,269

J. F. SCHEID ET AL

METHOD OF MAKING FINELY PERFORATED CERAMIC PLATES

Filed July 13, 1926



Fig. 1



Fig. 2



Fig. 3

Inventors:  
Johann Friedrich Scheid  
Viktor Sonnleitner

## UNITED STATES PATENT OFFICE.

JOHANN FRIEDRICH SCHEID, OF HERMSDORF, AND VIKTOR TONNDORF, OF JENA,  
GERMANY, ASSIGNORS TO THE FIRM: CARL ZEISS, OF JENA, GERMANY.

### METHOD OF MAKING FINELY-PERFORATED CERAMIC PLATES.

Application filed July 13, 1926, Serial No. 122,214, and in Germany January 24, 1925.

For various purposes, particularly for the manufacture of artificial fibres, e. g. artificial silk it is necessary to use plates with very fine openings. Such plates may be used as 5 filter plates, for instance, as sieve-plates for filtering the spinning material in the manufacture of artificial silk, or the openings of such a plate form the nozzles through which the spinning material is squirted. To re- 10 place the metal plates customary for these purposes by ceramic plates proved difficult because it was not possible to make in a simple way plates which with regard to the quality of the execution of the holes satisfy 15 the high demands which one is bound to make.

According to the present invention these plates are made in such a way that one forms the respective plate of ceramic material and 20 provides the still plastic plate with the desired holes by piercing the plate. In order to attain that in the finished plate the holes have exactly the desired shape up to their extremity one suitably does not entirely 25 pierce the plastic plate but only sticks into it, hardens it (e. g. by burning) after the sticking-in and then removes the unpierced part of the plate. By means of steel needles it is thus possible to make holes of exceed-

ingly small diameter (smaller than 0,2 mm.) 30 which according to their shape and size exactly meet the requirements.

The accompanying drawing shows an example of the invention. Fig. 1 shows a longitudinal section through a semi-finished 35 spinning nozzle, Fig. 2 shows the appertaining plan, Fig. 3 shows the finished spinning nozzle in a longitudinal section.

Into the bottom of a body *a*, moulded of still plastic porcelain material, holes *d* are 40 made with the aid of needles *b*, which are fixed in a head *c*, in such a way as not to pass through the bottom (see Fig. 1). Thereupon the body is burnt and the bottom worked off corresponding to the line *X* *X*. 45 Thereby one obtains the finished spinning nozzle as shown in Fig. 3.

#### We claim:

Method of making finely perforated ceramic plates, consisting in this that a plate of ceramic material is moulded, thereupon holes stuck into the plate, which do not entirely traverse the plate, then the plate hardened and finally the part of the plate not traversed by the holes removed. 50

JOHANN FRIEDRICH SCHEID.  
VIKTOR TONNDORF.